

Patented July 7, 1925.

1,545,196

# UNITED STATES PATENT OFFICE.

HARRIE C. PIERCE AND CHAD H. HUMPHRIES, OF KOKOMO, INDIANA, ASSIGNEES TO  
JAMES CLARK PATTEN, OF KOKOMO, INDIANA.

## CHROMIUM PLATING.

No Drawing.

Application filed May 5, 1924. Serial No. 711,956.

To all whom it may concern:

Be it known that we, (1) HARRIE C. PIERCE, and (2) CHAD H. HUMPHRIES, citizens of the United States, residing at (1) Kokomo, (2) Kokomo, in the counties of (1) Howard, (2) Howard, and State of Indiana, have invented certain new and useful Improvements in Chromium Plating, of which the following is a specification.

10 This invention relates to the electrodeposition of chromium and more particularly to a process of electroplating chromium and to a bath or solution for use in connection therewith.

15 The electrolyte or bath most commonly used and described in the literature for the electrodeposition of chromium in the form of smooth adherent deposits is the so-called "Sargent's solution," an essential characteristic of which is that it contains chromic acid and a relatively small amount of chromic sulfate. The best results are obtained with this solution after it has been aged for a time by the passage of an electric current through it, and even then the results are erratic and undesirable at current densities less than about 40 amperes per square foot. Higher current densities in the neighborhood of 100 amperes per square centimeter ordinarily are recommended.

In accordance with the process of our invention the aging referred to is avoided and smooth adherent deposits are obtained at current densities as low as 14 amperes per square foot.

Our invention consists generally in preparing a bath containing essentially chromic acid, ammonium sulfate and hydrated chromic hydroxide dissolved preferably in distilled water and electrolyzing this solution using either a chromium or other suitable anode such as iron or lead and a steel, brass or other metal cathode upon which the chromium deposit is desired and a current density ranging from about 14 up to about 125 amperes per square foot.

50 The bath may be prepared in a variety of ways, for instance by dissolving chromic acid in water, preferably distilled, and mixing with this solution a solution prepared by dissolving chromic sulfate and a quantity of ammonium hydroxide sufficient to approximately quantitatively decompose the chromic sulfate in water. An example of a preferred composition and the preferred

method of preparing it in accordance with our invention is as follows: A solution is prepared by dissolving 2 pounds of chromic acid C. P. in  $\frac{3}{4}$  gallon of water, preferably distilled. A second solution is prepared by dissolving  $\frac{1}{2}$  ounce of chromic sulfate in  $\frac{1}{4}$  gallon of water and adding thereto 30 to 40 cc. of a 28% ammonium hydroxide solution. The second solution is mixed into the first giving a plating solution which is ready for use directly without aging. The density of the plating solution is about 20° Bé.

A solution so prepared has some of the characteristics of the so-called "Sargent's solution" after the latter has been aged, particularly in its appearance, being of a very dark color and opaque. It does not, however, require aging, and is ready for use directly as soon as it is prepared and it also differs from an aged "Sargent's solution" in that from it light, continuous, coherent and homogenous deposits apparently free from green chromium oxide can be produced at current densities as low as 14 amperes per square foot whereas in order to secure similar results with an aged "Sargent's solution" a current density of 40 amperes or more per square foot is necessary.

The composition of our plating bath may be varied within a rather wide range, the range of variation being somewhat greater than in the case of the "Sargent's solution." The chromic acid content of the bath may vary from 80 to 450 grams per liter. The quantity of chromic sulfate used in making up the bath preferably amounts to from 1 to 2% of the chromic acid content. The preferred amount of ammonium hydroxide is the amount just sufficient to react with the chromic sulfate or only slightly in excess of that amount. The effect of the ammonium hydroxide appears to be analogous to that produced by aging, this effect being secured in a degree proportional to the relative quantity used up to a quantity equivalent to the chromic sulfate. Consequently it is within the scope of our invention to use any substantial quantity of ammonium hydroxide less than the chemical equivalent of the chromic sulfate used for the purpose of securing a corresponding effect. Or considering the solution of our invention as a solution of chromic acid, ammonium sulfate and hydrated chromic hydroxide with or

100  
105  
110

without chromic sulfate, it is within the scope of our invention to vary the quantities of ammonium sulfate and chromic sulfate, the former from a quantity chemically equivalent to the hydrated chromic hydroxide content of the bath, down to the smallest substantial quantity capable of producing a beneficial effect, and the latter in inverse ratio.

10 The best temperature of operation is at about room temperature and should not ordinarily exceed 80° F.

As is stated above, either metallic chromium or an inert anode may be employed

15 but chromium is preferred since its use tends to maintain the composition of the bath. The composition of the bath is not, however, completely maintained by the use of a chromium anode and it is necessary in order to

20 maintain the composition of the bath to add to it chromic acid in quantity sufficient, as may be determined by analysis, to maintain the chromium content thereof.

The current density employed in the elec-

25 trodeposition, as has been stated, may vary from as low as 14 amperes per square foot to 125 amperes or more per square foot, good deposits being obtained throughout this entire range. For commercial electro-plating

30 for protective and ornamental purposes the lower current densities, say from 14 to 40 amperes per square foot, are preferred since within this range it is possible to continuously produce smooth, continuous, adherent

35 deposits of a good white color. With the lower current densities the current efficiency is low, but due to the nature of the deposits, they being continuous, coherent, dense and hard, very thin deposits are sufficient. A

40 deposit .00015 inches or less thick such as may be produced in less than an hour with a current density of 25 amperes per square foot constitutes a commercial coating for many finishes on steel, iron, brass and copper.

45 Chromium coatings produced in accordance with our invention of from .00005 to .0002 inches in thickness compare favorably with standard nickel coatings which are from about .0003 to .0006 inches thick. The chromi-

50 um coatings are highly protective due to their hardness and to the fact that they are more continuous (have less pin holes) than other common coatings, for instance nickel coatings. Coating .0002 inches thick have

55 been found to be resistant to acid fumes, atmospheric corrosion, nitric and sulfuric acids and to tests involving the alternate wetting and drying of the coatings for a period of several months. The coatings have a very high luster, they can be polished by means of a buff wheel and colored and they show no tendency to peel or crack.

60 The color of the deposits varies somewhat

with the current density employed in producing them from a bright tin white at low 65 current densities to a dark gray color at high current densities.

We claim:

1. A bath for the electrodeposition of chromium containing chromic acid and relatively small proportions of hydrated chromic hydroxide and ammonium sulfate in aqueous solution. 70

2. As a bath for the electrodeposition of chromium, an aqueous solution of the reaction products of chromic acid, chromic sulfate, and ammonium hydroxide. 75

3. As a bath for the electrodeposition of chromium, an aqueous solution containing from 80 to 450 grams of chromic acid per 80 liter, and the reaction products of chromic sulfate in quantity amounting to from 1 to 2% by weight of the chromic acid content of the solution and ammonium hydroxide in quantity substantially chemically equivalent 85 to the chromic sulfate.

4. A bath for the electrodeposition of chromium produced by mixing a solution of the reaction products of chromic sulfate and ammonium hydroxide with a solution of 90 chromic acid. 90

5. Process of electrodepositing chromium which comprises passing an electric current in a circuit comprising an anode, a cathode and a bath containing chromic acid, hydrated chromic hydroxide and ammonium sulfate. 95

6. Process as defined in claim 5 in which the anode is metallic chromium.

7. Process as defined in claim 5 in which 100 the composition of the bath is maintained by the addition of chromic acid.

8. Process as defined in claim 5 in which a current density of from 14 to 125 amperes per square foot is employed. 105

9. Process as defined in claim 5 in which a current density of 14 to 40 amperes per square foot is employed.

10. Process of electrodepositing chromium which comprises passing an electric current at a current density of from 14 to 40 amperes per square foot through a bath containing from 80 to 450 grams of chromic acid per liter and the reaction products of chromic sulfate in quantity amounting to 110 from 1 to 2% by weight of the chromic acid content of the bath and a chemically equivalent quantity of ammonium hydroxide maintained at a temperature not over 80° F. between an anode of metallic chromium and 115 a cathode of a metal to be electro-plated. 120

In testimony whereof, we affix our signatures.

HARRIE C. PIERCE.  
CHAD H. HUMPHRIES.